

## UNITED STATES PATENT OFFICE

HERBERT WITTEK, OF BEUTHEN, GERMANY

## PROCESS OF REDUCING ORES

No Drawing. Application filed December 1, 1926, Serial No. 152,069, and in Germany July 26, 1926.

During the azotizing of carbides considerable quantities of heat are liberated which have, hitherto, been utilized only partly, for instance, for heating to the reaction temperature other masses of carbide yet to be nitrogenized. At the nitration of calcium carbide for instance, the exothermal heat generated usually causes superheating, and consequently decomposition of the nitro-lime which is formed, and thus prevents complete utilization of the carbide. During the nitration as well as at the preliminary heating of the carbide, carbon and hydrogen and other reducing gases are liberated which get lost without being utilized.

It has been ascertained by experiments that the heat liberated at the azotizing of carbide, as well as carbide which remains non-utilized at the usual azotizing, and also the above mentioned liberated substances may be advantageously utilized for the reduction of ores, if the reduction is made to take place in combination with the azotizing of carbides. Evidently only such compounds can be utilized during the nitration which do not prevent nitrogen binding with the carbide.

Ores the metals of which separate by distillation at the temperatures in question are specially adapted for the process. The process is very advantageous for the production of nitro-lime from calcium carbide. The ore admixed with carbide, or alternating layers of ore and carbide can be reduced in the oven at the same time that the nitration is taking place. In this manner the disagreeable effects of superheating are avoided, which otherwise occur during nitration by known methods, whereas in the present process the liberated heat is utilized at once for the reduction of the ores. The liberated carbon and gases exert further a strong reducing effect which is further favored by the carbide remainder the azotizing of which has, up to the present, been very difficult.

For this process zinc ores, for instance calamine, are specially adapted. When a mixture of calamine and carbide is used, the reduction of the zinc ore takes place in the oven together with the formation of nitro-lime, the zinc being separated by distillation

and obtained in a condensing plant. If sulphurous ores are used carbonic disulphide is produced in the oven which can be isolated from the gases of reaction in the well known manner.

The nitro-lime which is obtained by the nitration of calcium-carbide by nitrogen or ammonia according to the present process is superior to the nitro-lime obtained by the hitherto applied process, for the reason that it is practically free of carbide. The nitro-lime is delivered from the oven not in the form of a solid block, but in the form of a loose mass, as fusion of the mass does not take place owing to the suppression of the superheating. It is consequently not necessary to pulverize the mass to the usual state of dust for producing an effective fertilizer.

It is also possible to proceed in such a manner that the carbide admixed with ore or covered by ore is first brought to reducing reaction temperature in a stream of nitrogen by direct heating of the carbide, with the consequent production of reducing gases. After the reduction, the nitrogen then begins to act upon the carbide in the heated state. The advantage is thus obtained that the gases capable of reaction with the ore, generated at the heating of the carbide, which are otherwise lost, are utilized for the reduction of ores.

The reduction of the ores could also be carried out in a special oven, only the quantity of heat which is liberated at the azotizing of carbide being used for heating and reducing the ores, or the reduction of the ores may be carried out in a special oven, the gases liberated at the heating of the carbide and at the azotizing being used as reduction means.

If the object is to obtain only a carbide-free nitro-lime the reduction of the ores can be utilized to produce from raw nitro-lime a carbide-free calcium nitrogen, by bringing to reaction with the ores to be reduced the pulverized raw nitro-lime which still contains free carbide.

Instead of carbide, mixtures of carbide forming elements might evidently be used for the azotizing process without altering the process. To the carbide, as well as to the mix-

tures of carbide forming elements, the known additions, as calcium chloride, calcium fluoride, sodium chloride or the like, may be added which reduce the reaction temperature or accelerate the reduction.

Instead of calcium carbide, other carbides may be used for the reduction of the ores, for instance barium carbide. In this case barium cyanide is almost exclusively obtained. If strontium carbide is used, mixtures of the cyanide and of the cyanamide are obtained. When cyanides are formed the portion of the carbon of the carbide used for the binding of the cyanide is not at disposal for the reduction.

The quantity of carbide consumed in the reduction process can be reduced by adding at the same time coke to the carbide. The coke is either mixed with the carbide or placed in layers upon the carbide. Semi-coke is specially adapted as an addition, as it generates, prior to and at the occurring reduction temperatures of 800 to 1100° C., considerable quantities of hydrogen, the good effect of which at the reduction is generally known. By the addition of semi-coke the consumption of carbide for the reduction process is reduced and the lucrativeness of the process increased.

The invention has numerous applications, some examples of which are as follows:

A mixture of 170 parts by weight of carbide with 12 parts by weight of pyrite is heated in nitrogen gas to 1100° C. and nitrated as usual. The residue contains a calcium cyanamide of about 20% nitrogen and also the iron in finely divided metallic form. After comminution of the reaction product, the iron may be separated from the calcium cyanamide by washing, or by means of an electromagnet.

A mixture of 170 parts by weight of calcium carbide with 13.5 parts by weight of roasted blonde is heated to 1000°-1100° C. and treated with nitrogen. As soon as the nitration is completed and while nitrogen is passed through the same, the mass is allowed to cool. A calcium cyanamide of 20% nitrogen is obtained; it contains only a trace of zinc dust. In the receiver from 80 to 90% of the zinc is held in solid form. The rest is obtained from the waste gases by a dust removing device.

The carbide exposed to nitration is covered with a layer consisting of 100 parts of cinnamon bar and 100 parts of coke. By direct heating the carbide is first brought to the reaction temperature in the stream of nitrogen. The gases escaping penetrate the covering layer, and reduce part of the mercury ore, which by the heated carbide, is gradually brought to the reaction temperature. As soon as the nitration reaction sets in, through the heat thereby released and also with the help of the reducing gases formed therein, the remainder of the mercury ore is reduced, and

in consequence of the vapor stream, the mercury is driven out of the ore coke mixture, practically without residue. The volatile mercury is obtained as usual by a condensation pipe system, cooled by air and water, partly as a fluid mass and partly as the so-called mercurial soot.

I claim:

1. The method of reducing ores which consists in contacting the ore and carbide, and then azotizing the carbide, while the ore and carbide are thus associated.

2. The method of reducing ores which consists in mixing the ore and carbide, and then azotizing the carbide.

3. The method of reducing ores which consists in mixing the ore, a carbide and a semi-coke, and then azotizing the carbide.

4. The method of reducing ores which consists in passing a stream of nitrogen through a mass composed of alternating layers of ore and a carbide, heating the mass, whereby nitration of the carbide is effected, and recovering the metal of the ore liberated by the products of nitration.

5. The method of reducing ores which consists in azotizing a mass composed of the ore and calcium carbide, whereby a nitro-lime is formed and heat evolved, and separating the metal from the ore by means of the evolved heat.

6. The method of reducing ores which consists in forming a mixture of the ore and carbide containing compounds, and then azotizing the carbide.

7. The method of reducing ores which consists in forming a mixture of the ore and carbide forming elements, heating the mixture to form carbides, azotizing the carbides, and reducing the ore by means of the evolved gases.

8. The method of reducing ores which comprises forming a mixture of ore and nitro-lime containing carbide compounds, then reducing the ore by the carbide, whereby a pure nitro-lime is obtained and the ore is reduced.

In testimony whereof I affix my signature.

HERBERT WITTTEK.